

March 16, 1937.

J. W. YAXLEY

2,073,821

MANUFACTURE OF TIRE CORDS

Filed Oct. 6, 1933



FIG.1



FIG.2

FIG.3



Inventor  
J. W. Yaxley  
By E. F. Goddard & Son, Attorneys

## UNITED STATES PATENT OFFICE

2,073,821

## MANUFACTURE OF TIRE CORDS

John William Yaxley, Montreal, Quebec, Canada, assignor to Drummondville Cotton Company, Limited, Montreal, Quebec, Canada

Application October 6, 1933, Serial No. 692,390

3 Claims. (Cl. 117—52)

The invention relates to the manufacture of tire cords, as described in the present specification and illustrated in the accompanying drawing that forms part of the same.

5 The invention consists essentially in producing from fibers of different species, the finished product, as pointed out in the claims for novelty following a description in detail of a method of including the fireproof fiber in the yarn and subsequent cord.

10 The objects of the invention are to construct a tire cord that will eliminate to the greatest extent possible the dangers incident to the working of the cords in what are familiarly and commonly termed cord tires otherwise to furnish to the public a heat resisting element in the tire that will ameliorate the bad effects of friction and generally to provide for vehicle tires, efficient and durable cords.

15 In the drawing, Figure 1 is a diagram or table of the customary steps to produce a cord.

Figure 2 is a fragmentary sectional perspective view of a tire showing a cord withdrawn.

20 Figure 3 is an exaggerated detail of a piece of cord partially undone to disclose the strands and threads and showing the asbestos fibres intermingling with the cotton.

25 Like numerals of reference indicate corresponding parts in the various figures.

30 Referring to the drawing, the finished cords indicated by the numeral 15 have the same appearance as tire cords presently manufactured from cotton and other material, but in the beginning of the process, the lap in the scutching step is a thorough mixture of raw cotton fiber and raw asbestos fiber, and following the scutching, this lap or mixture of cotton and asbestos is carded preferably by a carding machine that is more suitable to the manufacture of wool

35 yarns.

40 After the carding the drawers operate, then the slubber, intermediate and roving frames are used in the reduction of the thickness of the sliver, the evenness of the product, the twisting of the roving and the winding of the roving on the bobbin, and following this, the spinning machinery completes the attenuation of the roving so far as to form a thread or yarn and twist the yarn that is thus formed, and give it the required strength.

45 The name "ply yarn" is given to all threads that are composed of two, three or more single yarns, twisted together at one operation and these yarns all contain the asbestos fiber introduced in the cotton fiber, and when thus indis-

criminately mixed together, they are distinguished from one another by the terms "two ply", "three ply" and so on, and when two or more ply threads are twisted together, the resulting yarns are spoken of as "cabled yarns" and the required strength having been reached, the plies of cotton and asbestos constitute the cords.

5 Usually these cords are woven into margins at the ends and in between these margins occasional weft threads are introduced there across.

10 This is of course common practice, except for the asbestos, and the quantity of this asbestos in proportion to the quantity of the cotton is all a matter of judgment in so far as the manufacture is concerned, but usually anything from thirty to fifty percent is considered sufficient to 15 resist overheating in the cords.

15 This must not be confused with asbestos cloth, which is not introduced in the same way, neither is the cotton in any quantity whatsoever, it is merely a binder in the asbestos web, usually there being approximately 90% of asbestos and 10% of cotton or even less of the cotton and made by an entirely different process. It must be remembered that the present invention is a composite cord made up of several strands which in themselves are composite being composed of mixed asbestos fibers and cotton filaments drawn out from the fibrous materials, which means that considerable tensile strength is maintained and this makes the cords desirable for reinforcement in building up tires and not to be compared or confused with woven fabrics. The cord itself is the invention and not the manner of installation because the task of introducing into a tire structure may be varied and in any event is largely conventional.

20 These cords have been indicated by the numeral 15 in the drawing while the numeral 16 indicates the strands of the cord. The threads forming the strands are indicated by the numeral 17. The asbestos fibers 18 are shown as intermingling in the body of the cotton, although in the cord itself the asbestos fibers are indistinguishable from the cotton so far as general appearance is concerned, the asbestos presenting here and there parts of the fibers on the surface of the cord which resist the heat and insulate the cord from the heat produced by friction which would otherwise tend to destroy the cord.

25 What I claim is:—

30 1. A composite tire cord made up from the 35 yarns resulting from the carding of a lap composed of a thorough mixture of cotton and asbestos fibers.

2. A composite tire cord made up from yarns emanating from a ready mixed lap having a predominance of cotton fibers heatproofed by the asbestos fibers that complement the cotton.
- 5 3. A composite tire cord made up from the yarns resulting from the carding of a lap com-

posed of a thorough mixture of cotton and asbestos fibers said asbestos fibers presenting heat resistant elements to the surface of the cord when the yarns are twisted.

**JOHN WILLIAM YAXLEY.**